

1

3,396,108

**EXTREME PRESSURE SOAP AND COMPLEX THICKENED GREASES**

Gerard P. Caruso, New Orleans, La., assignor to Shell Oil Company, New York, N.Y., a corporation of Delaware  
No Drawing. Filed Dec. 22, 1964, Ser. No. 420,425  
7 Claims. (Cl. 252—18)

This invention relates to non-clay thickened grease lubricants having improved extreme-pressure properties. More particularly, the invention relates to certain soap- and complex-thickened greases which are improved with regard to their ability to lubricate properly under extreme pressure (EP) conditions.

Prior to about 1940, nearly all grease requirements were met with uninhibited mineral oil thickened with calcium, sodium, or aluminum soaps. However, in the early 1940's the discovery of lithium soap thickened greases led to the development of water-resistant greases having high melting points and superior low-temperature properties. Later, in the 1950's, the discovery of lithium hydroxystearate-thickened greases paved the way for multi-purpose greases having excellent shear stability coupled with water resistance and good high- and low-temperature properties. In the late 1950's the need by industry and the armed forces for improved performance at temperatures ranging from —100 to +600° F. led to the development of many new types of oils, thickeners and additives.

While new thickeners, particularly waterproofed clays, have opened new vistas of grease performance, soap-thickened and complex-thickened greases still represent by far the major part of grease production and use in the world.

One of the major problems in the formulation of greases, particularly non-clay-thickened greases, is that of extreme-pressure (EP) properties, that is, the formulation of greases which have high film strength under high pressures. Literally thousands of materials of highly varying degrees of effectiveness, have been proposed to improve the EP properties of conventional greases. Among the many types of EP additives are sulfur, selenium and tellurium compounds, metal chlorides and sulfides and the like. In particular, certain metal sulfides, which are themselves good solid lubricants having EP properties, have been suggested for incorporation into grease. Among the metal sulfides which have been tried are antimony sulfide, molybdenum sulfide and zinc sulfide. However, such metal sulfides have not generally been found to be satisfactory EP agents in grease without the use of other additives to reduce the abrasiveness of such materials. For example, it is disclosed in U.S. 2,285,739 to use lead naphthenate in conjunction with zinc sulfide to reduce the abrasiveness of the metal sulfide. However, despite the extensive work on the use of metal sulfides in grease, the degree of EP effectiveness heretofore attainable in view of the cost of such lubricants, has not been sufficient to bring about their widespread application. Though, recently, waterproofed clay-thickened EP greases containing amorphous metal sulfides (antimony or molybdenum) have become available and are gaining increasingly wide acceptance, soap- or complex-thickened greases having comparable EP properties have been hitherto unobtainable.

However, applicant has now discovered that soap or complex greases having excellent EP properties can be made economically by incorporation therein of amorphous antimony trisulfide. More particularly applicant's invention is a naphthenate-free grease composition consisting essentially of (1) a lubricating base oil containing minor amounts each of (2) an oil-soluble sulfonate corresponding to the formula

2

wherein A is selected from the group consisting of alkali metal, alkaline earth metal, ammonium and omega-amino alkyl ammonium, n equals the valence of A and R is a monovalent hydrocarbyl radical selected from the group consisting of alkyl, aryl, alkaryl or aralkyl groups containing at least 6 carbon atoms, and (3) a metal sulfide primary EP agent, the lubricating oil being thickened to grease consistency by means of a soap-base thickening agent.

By the term "soap-base thickening agent," as used herein, is meant metal soaps of fatty acids which are capable of providing a stable gel structure to lubricating base oils. The term is intended to include conventional metal soaps, complex soaps, mixed base soap greases, and the like, and includes the following particular types of soap thickeners:

Metal base:

Aluminum base  
Barium base  
Calcium base  
Lithium base  
Sodium base  
Lead soap base  
Strontium base

Mixed bases:

Sodium-calcium base  
Sodium-barium base  
Calcium-aluminum base  
Sodium-aluminum base  
Magnesium-aluminum base  
Lithium-aluminum base

Metal complex:

Hydrated calcium soap  
Hydrated aluminum soap  
Hydrated barium soap  
Hydrated lithium soap  
Hydrated sodium soap  
Hydrated strontium soap  
Complex aluminum soap  
Complex barium soap  
Aluminum-barium complex  
Aluminum-sodium complex  
Complex calcium soap  
Calcium soap-calcium acetate complex  
Calcium soap-calcium chloride complex  
Calcium soap-strontium hydrate complex  
Calcium-barium soap complex  
Lithium soap-lithium acetate  
Magnesium soap complex  
Lead soap complex  
Sodium soap-sodium acetate complex  
Sodium soap-sodium acrylate complex  
Sodium-barium complex  
Strontium-calcium acetate complex

Though the lubricating base oil component of the invention can be either a natural or synthetic oil, as a practical matter, the base oil will usually be a natural oil, e.g. a petroleum-derived mineral oil. Many synthetic oils such as silicone oils and various esters can be thickened effectively with soap thickeners; however, the thermal stability of soaps is usually considerably lower than the synthetic oils. Therefore there is usually no point in using expensive synthetic oils with soap greases. Exceptions to this, however, are some of the complex greases which possess considerably higher thermal stability than the conventional soap-base greases.

The sulfonates which are useful in accordance with the invention are the salts of alkali metals or alkaline earth metals and oil-soluble monosulfonic acids. These are frequently of petroleum origin. Examples of typical suitable sulfonates are given in the following table.

TABLE I.—ANALYSES OF TYPICAL SULFONATES

|                             | Sodium Petroleum Sulfonate | Calcium Petroleum Sulfonate | Barium Petroleum Sulfonate | Strontium Petroleum Sulfonate | Barium Naphthalene Sulfonate | Sodium Naphthalene Sulfonate | Ammonium Dinonyl Naphthalene Sulfonate | Ethylene Diamine Dinonyl Naphthalene Sulfonate |
|-----------------------------|----------------------------|-----------------------------|----------------------------|-------------------------------|------------------------------|------------------------------|----------------------------------------|------------------------------------------------|
| Sulfonate, percent wt.      | 62                         | 41                          | 40                         | 31                            | 50                           | 50                           | 50                                     | 50                                             |
| Mineral Oil, percent wt.    | 33                         | 58                          | 59                         | 68                            | 46                           | 46                           | 46                                     | 46                                             |
| Water, percent wt.          | 5                          | >0.5                        | 1                          | <0.5                          | 1.0.2                        | 1.0.2                        | 1.0.2                                  | 1.0.2                                          |
| Inorganic Salt, percent wt. | None                       | 1                           | 1.5                        | 1                             | None                         | None                         | None                                   | None                                           |
| Molecular Weight            | 400/470                    | ca. 890                     | 980/1,010                  | —                             | 1,055                        | 482                          | 477                                    | 980                                            |

<sup>1</sup> Maximum.

The metals which can be used in the sulfonates are the alkali metals (Periodic Group IA) sodium and potassium and the alkaline earth metals (Periodic Group IIA), calcium, strontium and barium.

Within the context of the foregoing chemical structural formula



when A is omega-amino alkyl ammonium or alkyl ammonium, the alkyl portion thereof contains from 2 to 6 carbon atoms. A process for the preparation of sulfonates of this type is disclosed in U.S. Patent 2,764,548 issued Sept. 25, 1956. The ammonium sulfonic acid salts are prepared by reaction of the sulfonic acid with aqueous solutions of appropriate aliphatic or aryl primary, secondary or tertiary amines, e.g. dimethylamine, ethylenediamine, mono-, di- and triethyleneamine. The metal sulfides which are used as the primary EP agent in the grease composition of the invention include molybdenum disulfide, an amorphous antimony sulfide and mixtures thereof. The amorphous antimony sulfide is specified as contrasted to the crystalline antimony sulfides. The latter, normally obtained by the mining of certain minerals such as stibnite, actually causes abrasion of metallic parts. This may be due either to the extreme hardness of crystals or may be due to natural-occurring impurities such as silicates or silica present in the mineral. The amorphous antimony sulfides (e.g., antimony trisulfide, antimony tetrasulfide, or antimony pentasulfide and mixtures thereof) vary in color from yellow to gray but usually are some variety of red, dependent upon the precise means of preparation and more particularly upon the particle size of the amorphous sulfide. They are preferably obtained by precipitation of the antimony sulfide from an aqueous solution of a water-soluble antimony salt, such as antimony chloride, by treatment with a sulfide such as sodium sulfide or hydrogen sulfide.

The term "primary EP agent" is applied to the metal sulfides within the context of the invention; since, as will be shown by the following examples, the metal sulfides are substantially ineffective to improve the EP properties without the presence of the above-described sulfonates.

#### Example I

To a number of samples of lithium soap greases of varying composition were added small amounts of amorphous antimony trisulfide. The antimony trisulfide was thoroughly dispersed through the grease, after which each of the greases was subjected to the Timken Extreme Pressure Test (ASTM Bulletin 228, February, 1958, pages 28-31). As is shown by the following table, none of the soap greases containing amorphous antimony trisulfide exhibited any substantial increase in its load-carrying properties even at extremely high metal sulfide concentrations.

TABLE II.—EP PROPERTIES OF METAL SULFIDE-CONTAINING SOAP GREASES

| Sample Designation               | A       | B                  | C       | D       |
|----------------------------------|---------|--------------------|---------|---------|
| Antimony Trisulfide, percent wt. | 0.75    | 1.0                | 1.0     | 5.0     |
| Consistency:                     |         |                    |         |         |
| ASTM Penetration:                |         |                    |         |         |
| Unworked                         | 282     |                    |         |         |
| Worked                           | 271     |                    |         |         |
| NLGI Grade                       |         | No. 2 <sup>1</sup> | No. 2   | No. 2   |
| Timken EP Value, pounds          | Fail 20 | Fail 20            | Fail 20 | Fail 30 |

<sup>1</sup> ASTM penetration range, 265-295.

#### Example II

A further series of experiments was then run in which the greases to which the antimony trisulfide was added also contained a minor amount of an alkaline earth metal sulfonate, in this case calcium petroleum sulfonate. Some of these greases, all of which are commercially available lubricants, also contain minor amounts of naphthenic acids or metal naphthenates as indicated. The data show that the metal sulfides are quite effective to improve the EP properties of the soap base greases but (1) only in the presence of the metal sulfonates and (2) only so long as the grease is free of any naphthenic acids or naphthenates.

TABLE III.—EP PROPERTIES OF SOAP BASE GREASES CONTAINING METAL SULFIDE AND SULFONATES

| Formulation                              | E    | F    | G    | H    | I    | J    | K                | L    |
|------------------------------------------|------|------|------|------|------|------|------------------|------|
| Soap <sup>1</sup>                        | 9.1  | 8.8  | 8.8  | 8.6  | 9.1  | 9.0  | 8.6              | 8.5  |
| Lubricating Base Oil                     | 86.5 | 85.3 | 85.7 | 86.0 | 85.9 | 85.8 | 88.8             | 87.5 |
| Calcium Sulfonate                        | 2.8  | 2.8  | 2.8  | 2.9  | 2.9  | 2.9  | 2.1 <sup>2</sup> | 3.0  |
| Amorphous Sb <sub>2</sub> S <sub>3</sub> | 1.0  | 1.0  | 1.0  | 1.9  | 1.5  | 1.5  | 1.0              | 1.0  |
| Naphthenate                              | 0.1  | 0.1  | 0.6  | —    | —    | 0.2  | 0.6              | —    |
| Corrosion Inhibitor                      | 0.6  | 1.4  | 0.9  | —    | 0.6  | 0.6  | —                | —    |
| Other Additives                          | —    | —    | —    | —    | —    | —    | —                | —    |
| Timken EP Value, pounds:                 | —    | —    | —    | —    | —    | —    | —                | —    |
| Pass                                     | 40   | —    | —    | 25   | 50   | 20   | —                | 55   |
| Fail                                     | 45   | 20   | 20   | 30   | 55   | 25   | 20               | 60   |

<sup>1</sup> Soap of LiOH-H<sub>2</sub>O and hydrogenated fatty acids. All formulations given on percent weight basis.

<sup>2</sup> Ethylene diamine dinonyl naphthalene sulfonate.

It is interesting to note from the above data (Formulation H) that even increasing the amount of metal sulfide failed to overcome the adverse effect of the presence of even a small amount of naphthenate.

The above data, Formulations K and L, indicate that the interaction of amorphous metal sulfides with sulfonates is not restricted to metal sulfonates but applies to organic salts of sulfonic acids as well. This is confirmed in the following example.

#### Example III

50 In this test, ethylene diamine dinonyl naphthalene sulfonate was substituted for alkaline earth metal sulfonate in a lithium hydroxide monohydrate-hydrogenated fatty acids soap-thickened grease. The Timken EP test results clearly showed the interaction between the sulfonate and 55 the amorphous metal sulfide.

TABLE IV.—EP PROPERTIES OF SOAP BASE GREASES CONTAINING METAL SULFIDE AND NON-METAL SULFONATE

| Formulation                              | M    |
|------------------------------------------|------|
| Soap, percent wt.                        | 9.4  |
| Lubricating Base Oil                     | 88.1 |
| Amorphous Sb <sub>2</sub> S <sub>3</sub> | 1.0  |
| Non-metal Sulfonate                      | 1.5  |
| Timken EP Value, pounds:                 | —    |
| Pass                                     | 55   |
| Fail                                     | 60   |

65 The amounts of metal sulfide and metal sulfonates which are to be used in the soap EP greases of the invention can each be varied from about 0.5 to about 10.0%, 1 to 5% by weight of each being preferred. The ratio of sulfonates to metal sulfide does not appear to be critical.

#### Example IV

70 The quite unexpected interaction of the sulfonates and the amorphous metal sulfides is perhaps most graphically 75 illustrated in view of the facts (1) that the metal sulfide

has substantially no EP activity in soap greases without the sulfonates (see Table II) and yet (2) in clay-thickened greases, in which the metal sulfides have at least some EP effectiveness, the sulfonates apparently do not effectively interact with the amorphous metal sulfides. This is illustrated by the following comparative tests in which the Timken EP properties of two identical naphthenate-free clay-thickened greases containing equal amounts of  $Sb_2S_3$  were compared with and without 3.0% by weight of calcium petroleum sulfonates. The results were as follows:

TABLE V.—EP PROPERTIES OF METAL SULFIDE-CONTAINING CLAY-THICKENED GREASES

| Formulation                  | N    | O    |
|------------------------------|------|------|
| Clay-thickened Grease        | 96.5 | 99.5 |
| Amorphous $Sb_2S_3$          | 0.5  | 0.5  |
| Calcium Petroleum Sulfonates | 3.0  | None |
| Timken EP Value, pounds:     |      |      |
| Pass                         | 40   | 40   |
| Fail                         | 45   | —    |

In the following table, a number of different grease formulations within the scope of the invention are exemplified.

2. The composition of claim 1 in which the mixture (3) consists of (a) calcium petroleum sulfonates and (b) amorphous antimony trisulfide.

3. The composition of claim 1 in which the mixture (3) consists of (a) sodium petroleum sulfonates and (b) amorphous antimony trisulfide.

4. The composition of claim 1 in which the mixture (3) consists of (a) omega-amino- $C_{2-6}$ -alkyl ammonium alkaryl sulfonate and (b) amorphous antimony trisulfide.

5. The composition of claim 1 in which the mixture (3) consists of (a) ammonium alkaryl sulfonate and (b) amorphous antimony trisulfide.

6. A soap base grease composition having improved extreme pressure properties consisting essentially of (1) a lubricating base oil thickened to grease consistency with (2) a thickening amount of the lithium soap of 12-hydroxy stearic acid and (3) a mixture containing 0.5–10.0% by weight, basis total composition, each of (a) calcium petroleum sulfonates and (b) amorphous antimony trisulfide, the composition being further characterized as containing no naphthenate compounds.

7. A soap base grease composition having improved extreme pressure properties consisting essentially of (1)

TABLE VI.—SOAP BASE EP GREASES CONTAINING METAL SULFIDES AND ALKALI- OR ALKALINE EARTH-METAL SULFONATES

| Lubricating Base Oil, percent wt.                                     | Thickening Agent |                                                   | Metal Sulfide  |                         | Sulfonate      |                                   |
|-----------------------------------------------------------------------|------------------|---------------------------------------------------|----------------|-------------------------|----------------|-----------------------------------|
|                                                                       | Percent weight   | Type                                              | Percent weight | Type                    | Percent weight | Type                              |
| 500 SSU at 100° F. Neutral Oil:                                       |                  |                                                   |                |                         |                |                                   |
| 82.0                                                                  | 10.0             | Aluminum soap of dimerized fatty acids.           | 5.0            | Amorphous $Sb_2S_3$ ... | 3.0            | Sodium petroleum.                 |
| 88.5                                                                  | 10.0             | do                                                | 1.0            | do                      | 0.5            | Calcium petroleum.                |
| 82.85                                                                 | 12.1             | Calcium 12-hydroxystearate                        | 0.05           | do                      | 5.0            | Do.                               |
| 85.0                                                                  | 11.0             | do                                                | 1.0            | do                      | 3.0            | Barium petroleum.                 |
| 87.2                                                                  | 8.8              | Barium soap of hydrogenated castor oil.           | 1.0            | do                      | 3.0            | Do.                               |
| 84.4                                                                  | 10.6             | Barium and calcium soap of fatty acids.           | 1.0            | $MoS_2$                 | 4.0            | Potassium petroleum.              |
| 70/30 mixture of 750 SSU at 100° F. red oil and 150 HV1 bright stock: |                  |                                                   |                |                         |                |                                   |
| 84.6                                                                  | 11.2             | Hydrated calcium soap of palm oil                 | 1.5            | $MoS_2$                 | 2.7            | Sodium petroleum.                 |
| 84.3                                                                  | 12.4             | Calcium soap of lard oil                          | 2.0            | $MoS_2$                 | 1.4            | Calcium petroleum.                |
| 90.45                                                                 | 6.3              | Calcium acetate—calcium soap complex.             | 0.05           | Amorphous $Sb_2S_3$     | 3.2            | Do.                               |
| 88.9                                                                  | 9.1              | Lithium soap of hydrogenated castor oil.          | 1.0            | do                      | 1.0            | Barium petroleum.                 |
| 81.5                                                                  | 13.3             | Lithium and aluminum soap of stearic acid.        | 1.0            | do                      | 4.2            | Strontium petroleum.              |
| Pentaerythritol esters: 83.8                                          | 10.2             | Sodium soap of 12-hydroxystearic acid.            | 1.0            | do                      | 5.0            | Barium dinonyl naphthalene.       |
| Silicone Oil: 86.3                                                    | 9.7              | Complex lead—sodium fish oil soap.                | 2.0            | do                      | 2.0            | Sodium petroleum.                 |
| 75 SSU at 210° F. neutral oil:                                        |                  |                                                   |                |                         |                |                                   |
| 85.0                                                                  | 11.0             | Sodium soap of tallow fatty acids                 | 2.0            | do                      | 2.0            | Do.                               |
| 82.0                                                                  | 10.0             | Mixed magnesium and aluminum 12-hydroxy stearate. | 5.0            | do                      | 3.0            | Calcium petroleum.                |
| 87.5                                                                  | 8.5              | Lithium soap of hydrogenated castor oil.          | 1.0            | do                      | 3.0            | Ethyl ammonium $C_{18-18}$ alkyl. |
| 87.5                                                                  | 8.5              | do                                                | 1.0            | do                      | 3.0            | Ammonium dioctyl naphthalene.     |

I claim as my invention:

1. A soap base grease composition having improved extreme pressure properties consisting essentially of (1) a lubricating base oil thickened to grease consistency with (2) a thickening amount of metal-containing soap, and (3) a mixture containing 0.5–10.0% by weight, basis total composition, each of (a) an oil-soluble sulfonate corresponding to the formula



wherein A is selected from the group consisting of alkali metal, alkaline earth metal, ammonium and omega-amino- $C_{2-6}$ -alkylammonium, n equals the valence of A and R is a monovalent hydrocarbyl radical selected from the group consisting of alkyl, aryl, alkaryl and aralkyl containing at least 6 carbon atoms, and (b) a metal sulfide selected from the group consisting of an amorphous antimony sulfide and molybdenum disulfide; the composition being further characterized as containing no naphthenate compounds.

60 a lubricating base oil thickened to grease consistency with (2) a thickening amount of the lithium soap of 12-hydroxy stearic acid and (3) a mixture containing 0.5–10.0% by weight, basis total composition, each of (a) ethylenediamine dinonylnaphthalene sulfonate and (b) amorphous antimony trisulfide, the composition being further characterized as containing no naphthenate compounds.

#### References Cited

#### UNITED STATES PATENTS

|           |        |                   |          |
|-----------|--------|-------------------|----------|
| 2,421,543 | 6/1947 | Cook              | 252—18   |
| 2,511,250 | 6/1950 | Fawcett           | 252—33.2 |
| 2,540,533 | 2/1951 | Kolfenbach et al. | 252—33.2 |
| 2,540,534 | 2/1951 | Kolfenbach et al. | 252—33.2 |
| 2,764,548 | 9/1956 | King et al.       | 252—33   |
| 2,846,392 | 8/1958 | Morway et al.     | 252—39   |
| 3,015,623 | 1/1962 | Loring et al.     | 252—18   |
| 3,269,947 | 8/1966 | Swenson           | 252—33.2 |

(Other references on following page)

## OTHER REFERENCES

"Petroleum Refining with Chemicals" by Kalichevsky et al., Elsevier Pub. Co., New York, 1956, p. 582.

"Manufacture and Application of Lubricating Greases" by Boner, Reinhold Pub. Corp., New York, 1954, pp. 760, 761, 781, 782.

"Advances in Petroleum Chemistry and Refining" by Kobe et al., Interscience Pub., New York, 1964, pp. 127, 128.

5 DANIEL E. WYMAN, *Primary Examiner.*  
I. VAUGHN, *Assistant Examiner.*